

## UNITED STATES PATENT OFFICE.

ERNEST BERTSCH, OF HAGUENAU, FRANCE.

## SENSITIZING COMPOSITION FOR PREPARING BLUE-PRINT PAPER.

No Drawing. Application filed August 29, 1921. Serial No. 496,593.

(GRANTED UNDER THE PROVISIONS OF THE ACT OF MARCH 3, 1921, 41 STAT. L., 1313.)

*To all whom it may concern:*

Be it known that ERNEST BERTSCH, citizen of France, residing at Haguenau, Alsace, France, has invented certain new and useful Improvements in Sensitizing Composition for Preparing Blue-Print Paper (for which I have filed applications in Germany, July 6, 1918; application of addition February 9, 1921; France, March 31, 1921; Denmark, March 30, 1921; Sweden, March 31, 1921; Norway, March 31, 1921; Holland, March 31, 1921; and Luxembourg, April 9, 1921), of which the following is a specification.

15 It is well known that in the production of blue negative light printing papers by the use of ferric salts for example alkali ferric oxalates to add thereto free oxalic acid so as to permit the white lines to appear more clearly. This result however is not obtained, but the paper thus produced possesses a series of disadvantages which exclude its possibility as a marketable article. The paper appears grey running into blue and deteriorates rapidly, therefore does not possess any durability. After exposure it does not give pure white lines. During exposure the tone passes from olive green to a dark shade of blue, dark indigo blue to grey blue; when washed the print becomes dark blue and white lines appear which in consequence of the dark blue tone appear blue, but this is not the case. The dark blue colour tone returns when drying so that the print becomes still more intolerable. Paper thus obtained cannot be manufactured on a large scale as on the cylinder acid oxalate salts are deposited which can only be dissolved with difficulty and which tear the paper during its production and make it streaky. The process is therefore only of slight value as the paper prepared thereby must be exposed directly after its preparation as otherwise it would not produce satisfactory copies.

According to the present invention a neutral alkali oxalate is added to the ferric salt, preferably at a strength of 10-20%. As an example the following may be mentioned: to 10 kg. of alkali ferric oxalate—as substitute for ferric ammonium acetate—are added  $\frac{1}{2}$  kg. of potassium or sodium oxalate. This salt mixture is then dissolved in 20 to 30 litres of hot water and to the solution is

then added in the known manner a solution of potassium ferricyanide. The two solutions are mixed together and diluted to 16° Bé. Paper prepared with this possesses just the opposite properties to that which is obtained by the process hereinbefore described using free oxalic acid. The neutral oxalate salt has a preserving effect upon the ferric salts and prevents the reduction thereof in the dark whilst free oxalic acid has a reducing and therefore a decomposing effect. The preparation therefore retains its yellow colour unaltered and is durable. On exposure the colour tone passes from yellow to emerald green, a shade of blue, bright blue, yellow grey to a bright yellow grey. After washing the blue colour tone increases in intensity by drying. The lines become snow white on a deep blue ground.

According to the invention the process is carried on a further stage to that wherein 10 to 20% of neutral alkali oxalate is added to the ferric salts as above described in that mono-acidic oxalate is added whereby the neutral salt is contained in excess in the mixture whilst the acid salt forms only a fraction thereof. In this case the excess of neutral salt in comparison to the mono-acidic oxalate produces a preserving effect so that a separate oxidizing agent is unnecessary.

In preparing this mixture the operation is preferably such that oxalic acid is neutralized by means of alkali or alkali carbonate and then the excess of oxalic acid favourable to the process is added; for example 126 grams of oxalic acid are neutralized by means of alkali or alkali carbonate and then 20 to 25 grams of oxalic acid are added.

The same applies to the potassium salt, sodium salt ammonium salt and other easily soluble oxalate salts. Other acids may be used in place of the oxalate salts as addition to the neutral salts and produce a favourable result such for example as lactic acid, acetic acid tartaric acid citric acid. The same action is produced by the addition of inorganic acids and acid salts which are easily soluble. Neutral alkali salts of organic acids also produce a favourable result.

The process can be carried out on a large scale. It is also a complete substitute for the citric acid process which in consequence of

the high price and the difficulty in obtaining citric acid cannot be carried out effectively.

Having now particularly described and ascertained the nature of my said invention and in what manner the same is to be performed, I declare that what I claim is:—

1. A composition for use in the production of blue print paper, comprising organic ferric salts, and a neutral alkali oxalate.

2. A composition for use in the production of blue print paper, comprising organic ferric salts about ninety per cent, and a neutral alkali oxalate, about ten per cent.

In testimony whereof I hereunto affix my <sup>15</sup> signature in the presence of two witnesses.

ERNEST BERTSCH.

Witnesses:

FRANK A. KELLER,  
JOHN A. SCOTT.